

## UNITED STATES PATENT OFFICE

GEORGE D. BEAL AND ROB ROY MCGREGOR, OF PITTSBURGH, PENNSYLVANIA

## MANUFACTURE OF FELT

No Drawing.

Application filed December 19, 1928. Serial No. 327,178.

Our invention relates to the treatment of animal fibres; such as wool, cows' hair, etc., in preparation for its manufacture into felt. It has been developed in the treatment of fur, and in that application we shall describe it. The objects in view are improvement in the quality of the product, reduction in the cost of production, and avoidance of manufacturing conditions such as to affect the health of operatives. The preponderant use for fur felt is in the making of hats.

It has long been known that by boiling in dilute nitric acid, with the addition of a small quantity of grease, the felting property of fur may be improved; the felting operation may be expedited. About the year 1725 the discovery was made that if, before removal from the pelt, the fur be brushed with a dilute solution of nitric acid and mercuric nitrate, the felting property of the fur may be more greatly improved. The reagents so applied affect primarily and chiefly the extremities of the hairs, and incidentally cause them to become discolored. Because of the discoloration, the treatment is called carotting. It is a treatment which has continued in commercial use to the present day.

There are objectional features of the carotting treatment. The discoloration of the fur, which in the manufacture of white and light-colored felts is particularly undesirable, may be avoided only by the exercise of great care; the best results are obtained by holding this fur at least a month after treatment, to age, before being used in hat-making, and such delay is undesirable; furthermore, inequalities in periods of aging tend to result in lack of uniformity in quality; the mercury salt is expensive, and its provision adds much to the cost of hat-making; the mercury present in the form and quantity and under the conditions of operation requires great sanitary precautions attendant on its use. Nevertheless, the industry has

sought in vain the avoidance of these objections and difficulties.

We have discovered that by subjecting fur to the action of steam under pressure felting property may be imparted to it; we have discovered that fur which has been brushed with a dilute solution of nitric acid and mercuric nitrate may advantageously be subjected to the action of steam under pressure; and we have discovered that if the fur, while still on the pelt, be brushed with a solution of a salt which under the influence of water tends to break up, with the production of an acidic or an alkaline solution, and particularly if the so broken-up components be a weak base and a strong acid, and if the fur be then subjected to the action of steam under pressure, felting property in still greater degree may be imparted to it.

The effect, we have discovered, is that of hydrolysis. It may be gained by subjecting the fur to the action of steam under pressure, no other agent being present. The effect is, however, intensified if another agent be present. If that other agent be the solution of nitric acid and mercuric nitrate known to the art, the steam treatment permits the use of a weaker solution with which to brush the fur. There is gain then in saving of material and in the fact that the precautions which must be taken when mercury is used are less burdensome; and there are the further gains, that the tendency to discoloration is diminished, that aging is no longer necessary, and that better uniformity of product so is attained.

Preferably we employ a solution of a salt or salts other than salts of mercury manifesting the tendency which we have mentioned, the tendency to break up in the presence of water. A suitable salt of the character indicated is chloride of magnesium; another is chloride of aluminum; another is ferric nitrate. The common characteristic which these salts possess of breaking up in

the presence of water into a weak base and a strong acid will be recognized by the chemist. And other salts having the same characteristic will lie fairly within his knowledge and contemplation. Which salt will be chosen, among those theoretically available, will depend on practical considerations. We have indicated particular salts which, generally speaking, are practically available. Other salts which break up into a strong base and a weak acid—sodium acetate, sodium phosphate, and sodium bi-carbonate, for examples—may be used, though we prefer salts of the class first mentioned.

It is possible to use, instead of a solution of a salt, a solution of an acid alone or of a base alone, subjecting the fur, when application of the solution has been made, to the action of steam under pressure, as in the preferred procedure. And, as has been explained, the fur may, without preliminary application to it of any solution, be subjected immediately to the action of steam under pressure.

The procedure in which our invention resides may be carried out typically as follows. The fur while still on the pelt is brushed with a "one-normal" solution of chloride of magnesium; the pelt is dried; the fur is removed from the pelt; and then, within an autoclave, it is for the period of an hour and a half subjected to the action of steam at a pressure of 20 pounds. Being then dried and removed from the autoclave, the fur is ready for the felting operation.

We have given the steam pressure which we have found to be convenient to use, and the time which we have found to be requisite for treatment at that pressure. These figures are given by way of example. The invention is practiced in treatment with steam under pressure, and the time requisite for treatment will vary as the pressure varies, being greater if the pressure be less.

The operation is one which, under a steam pressure, of (say) twenty pounds, is fully accomplished in about an hour and a half; no period of aging is required. It is an operation which in every detail and circumstance may be minutely controlled; and, in consequence, uniformity of product is attainable.

The fact has been recognized that similar classes of fur, prepared in similar manner, may have different felting properties. This we have found to be due, in part at least, to the difficulty of maintaining complete control over every step of the process. Our method here described, being susceptible to much more accurate control, affords a much more uniform product.

A great difficulty in felt-making, as hitherto it has been conducted, is to cause the fur to "wet" thoroughly. Fur treated by our method here described will in felt manufac-

ture be found to be free of this difficulty; it "wets" easily.

In the practice of our invention, the steam treatment effects sterilization of the material, and this manifestly is a desirable condition.

In the practice of our invention, while we may use a solution of a mercury salt, we are not under the necessity of doing so, and preferably we do not employ such a solution. Thus we may wholly avoid the necessity of taking sanitary precautions such as have been alluded to; we avoid also the relatively great cost of a mercury salt. We avoid those variations in the quality of mercury-carroted fur which are due to variations in times of aging. In the practice of our invention the tendency of the fur to become yellow or otherwise discolored is diminished, and in the operation as we prefer to conduct it that tendency completely disappears. The fur after treatment does not require aging, but may be used at once; and, as we have said, since the operation is susceptible to exact control, it is capable of affording a uniform product.

We have described the removal of the fur from the pelt before subjecting it to the action of steam under pressure in the autoclave. It is permissible to subject the fur while still on the pelt to the steam treatment, and afterward to remove the fur. Alternatively, it is possible first to cut the fur from the pelt, immerse it in the solution, dry it, and then subject it to the steam treatment; or, it may when cut from the pelt be subjected immediately to the steam treatment. It will be understood that the method may in practice be modified in such details.

The felt produced in the practice of our invention takes dye in more uniform manner than does felt hitherto produced.

Our treatment with the advantages described has practical value in the preparation of fur for felting. It is applicable, and with like effect, to animal fibre of other particular kinds; to cow hair, for example, and to wool. Cow hair may be used as a filler in felt making, and when cow hair is to be so used, we recommend that it be treated in the manner described.

We claim as our invention:

1. The method of preparing animal fibre for felt-making which consists in subjecting it to the action of steam under pressure, together with an acidic hydrolytic agent.

2. The method of preparing animal fibre for felt-making which consists in subjecting it to steam under pressure, together with a substance which in the presence of steam affords acidic reaction.

3. The method of preparing animal fibre for felt-making which consists in subjecting it to steam under pressure, together with a salt which in the presence of steam affords acidic reaction.

4. The method of preparing animal fibre

for felt-making which consists in subjecting it to steam under pressure, together with chloride of magnesium.

5. The method herein described of preparing fur for felt-making which consists in brushing the fur while still on the pelt with a salt which in the presence of steam under pressure affords acidic reaction, drying the fur, and subjecting it to the action of steam under pressure.

10 In testimony whereof we have hereunto set our hands.

GEORGE D. BEAL.  
ROB ROY McGREGOR.

16

20

25

30

35

40

45

50

55

60

65